

March 30, 1937.

G. A. ALBERT

2,075,328

METHOD OF IMPREGNATING CELLULOSIC MATERIALS AND PRODUCT OF SAID METHOD

Filed Oct. 3, 1933



VOLUME CHANGE - WEIGHT CHANGE  
 $\frac{1}{16}$  Granite Fibre, Water Bath 25°C.

FIG. 1



SPECIFIC GRAVITY - TIME IMMERSED  
 $\frac{1}{16}$  Granite Fibre, Water Bath 25°C.

Impregnated to  
minimum specific  
gravity with  
waterproofing  
material.



FIG. 2

FIG. 3

INVENTOR.

GERARD A. ALBERT

BY

adCaesar  
Charles W. Rivise  
ATTORNEYS

Patented Mar. 30, 1937

2,075,328

# UNITED STATES PATENT OFFICE

2,075,328

## METHOD OF IMPREGNATING CELLULOSIC MATERIALS AND PRODUCT OF SAID METHOD

Gerard A. Albert, Kennett Square, Pa., assignor to National Vulcanized Fibre Company, Wilmington, Del., a corporation of Delaware

Application October 3, 1933, Serial No. 691,923

6 Claims. (CL 91—68)

This invention relates to methods of impregnating cellulosic materials and to the products of such methods.

The primary object of the invention is to provide a method of impregnating cellulosic materials such as paper with various impregnating agents so as to impart thereto certain desirable properties such as greater water resistance without at the same time impairing other desirable properties such as flexibility or pliability.

Another object is to produce an indurated fibre having a greatly decreased water absorption, but which retains substantially undiminished all the desirable qualities and characteristics usually ascribed to this type of material, particularly its flexibility or pliability.

The method of the invention is particularly adaptable to indurated fibre of the type generally known in the art as vulcanized fibre, fibre or leatheroid. This type of material is generally made by treating cellulosic material in the form of sheets or webs with parchmentizing or gelatinizing agents. The cellulosic material is usually, though not necessarily, an all cotton cellulose paper. Among the various parchmentizing or gelatinizing agents that have been used or suggested may be mentioned aqueous solutions of alkalis such as caustic soda, dilute acids such as sulphuric and nitric, metallic salts such as zincates, stannates, stannites, antimonates, aluminates and preferably zinc chloride.

The parchmentizing or gelatinizing agents serve to chemically hydrate, partially hydrolyze, gelatinize or parchmentize the cellulose fibre so that when the treated material is laminated and subjected to heat and pressure, it is caused to coalesce and become indissolubly united into a homogeneous multi-ply sheet. By leaching and "puring out" the treating agent and subsequently drying the sheet, a hardened horn-like material results having greatly improved characteristics as compared with the cellulosic material originally subjected to the chemical and physical treatment. Its toughness, hardness, elasticity, flexibility or pliability, dielectric strength and the fact that it is oil-proof, impervious to organic solvents and fairly resistant to mineral acids render it eminently suitable for many purposes, both mechanical and electrical. Vulcanized fibre as made by prior art methods has, however, one serious drawback or shortcoming which greatly limits its field of usefulness; it is far from being waterproof or impervious to water and steam. In fact, commercial samples of vulcanized fibre readily take up as much as 25% or more of their weight of water depending upon a number of factors including the quality of raw materials and conditions under which the chemical and physical treatments are carried out.

Prior attempts to render vulcanized fibre water

resistant have for the most part been based upon impregnation with waterproofing materials such as varnishes, resins, oils, etc. Vulcanized fibre is, however, practically impermeable to ordinary waterproofing materials and organic solvents which are generally used as vehicles for waterproofing materials and, hence, attempted impregnation usually results in thin superficial coatings or films of varnishes which are not durable or water resistant and on being abraded or broken allow the absorption of high percentages of water. Likewise, it is impossible to introduce waterproofing materials into vulcanized fibre by means of aqueous suspensions or emulsions, for vulcanized fibre is an unusually good filtering medium and merely absorbs the water, leaving the waterproofing material as a coating.

It has been suggested in British Patent No. 316,700 to I. G. Farbenindustrie Aktiengesellschaft that the waterproofing materials be introduced into the fibre in the form of aqueous solutions. This patent discloses a method which depends upon the marked avidity of vulcanized fibre for water and proposes to utilize aqueous solutions of certain types of synthetic resins which can be readily converted by means of heat and pressure to a water insoluble, water resistant form. According to the disclosure of the patent the fibre is immersed in the waterproofing solution until it will take up no more resin and the saturated material is subjected to heat and pressure to convert the resin to final form.

Extensive tests indicate that the process results in a product which is fairly water resistant, but which has totally lost the flexibility or pliability so characteristic of vulcanized fibre. The product has all the physical appearance of a board made by impregnating individual sheets of paper with synthetic resins and laminating the impregnated sheets with heat and pressure and is too brittle for the purposes for which vulcanized fibre is generally used.

The present invention depends upon the discovery that if a substantially flexible material, such as paper, vulcanized fibre, etc., is impregnated to substantially minimum specific gravity, not only will it acquire the desirable properties of the impregnating agent such as greater water resistance but it will also retain its own desirable characteristics such as flexibility.

In view of the fact that the invention is particularly well adapted for the preparation of water resistant vulcanized fibre, this material has been selected as the illustrative embodiment of the invention for the purpose of the present disclosure.

Referring briefly to the drawing, Figure 1 is a graph indicating the relationship between the increase in volume and the increase in weight of a sample of fibre immersed in water at 25° C.;

Figure 2 is a graph indicating the variation of the specific gravity of the sample of Figure 1 with time of immersion; and

Figure 3 is a cross-section through a laminated sheet of cellulosic material made according to the teachings of the present invention.

Briefly stated, the process of the present invention consists in immersing the vulcanized material until it attains minimum specific gravity, 10 drying, and subjecting the dried material to such treatment as is necessary to change the waterproofing material to its final water resistant form.

For the purposes of the present invention, any material may be used as the saturant or impregnating agent provided it is water-soluble at one stage and insoluble at another stage and provided further that in its insoluble stage it has pronounced waterproofing qualities. Among the materials fulfilling the required specifications may be 15 mentioned the modified natural or synthetic resins falling within the following groups:

(1) The water-soluble phenol-aldehyde type of resin such as is made by the Bakelite Corporation and sold under the designation "Bakelite Water Soluble Resin XR-568".

(2) The water-soluble aldehyde-ketone type of resin described in Patents Nos. 1,502,945 and 1,761,542 to Ellis granted July 29, 1924 and June 30, 1929, respectively.

(3) The water-soluble urea-formaldehyde and thiourea-formaldehyde types of resin such as are disclosed in Patent No. 1,507,624 to Pollak et al., dated September 9, 1924 and Patent No. 1,926,786 to Novotny et al., dated September 12, 1933.

(4) The water-soluble alkyd or glyptal type of resin described in Japanese Patent No. 93,029 to Habu, dated September 29, 1931 and abstracted in Chemical Abstracts, Volume 26 (1932), page 4488. This type of resin may be made by heating glycerol or glycol and citric or tartaric acid at 170-180° for 40 an hour and combining the resinous product with a fatty or aromatic acid, acetic anhydride, benzoic anhydride or alkyl iodide.

I prefer to employ the phenol-aldehyde type of resin, for generally speaking the phenol-aldehyde resins are the most easily convertible of all synthetic resins and for that reason lend themselves most readily to the purposes of the present invention. Bakelite Water-Soluble Resin XR-568 is 45 particularly suitable. This material is a water-soluble phenol-formaldehyde reaction product basically reacted. It is supplied by the manufacturer in a water solution and may be diluted to a resinoid content of approximately 30% without 50 signs of precipitating the resin. If greater dilution is desired, a small amount of alcohol may be 55 added to keep the resin in solution.

An explanation of minimum specific gravity will 60 now be given. When a dry piece of vulcanized fibre is immersed in water, it immediately takes up water and begins to swell. A close study of this 65 swelling with water absorption reveals the fact that the change in volume of the piece (the swelling) is directly proportional to the weight of the water absorbed. This proportionality is interpreted as meaning that the water absorbed into the body of the fibre is at once taken up by the cellulose which swells in proportion to the amount 70 of water taken up. As more and more water is absorbed, the cellulose becomes saturated and it can no longer expand proportionately, with the result that the linear relation between volume change and weight change ceases. Beyond this 75 point, the water that is absorbed into the body of

the fibre goes to fill the interstices of the material with consequently a slight change in the over-all volume of the sample. The graph of Figure 1 illustrates the foregoing explanation, the sample being a piece of granite fibre having a thickness of  $\frac{1}{8}$ ".

Specific gravity determinations made at the same time reveal that the specific gravity of the sample decreases very rapidly at first, reaches a minimum and then increases but gradually. The variation of specific gravity with time of immersion is indicated on the curve of Figure 2. The important connection between the two graphs is that minimum specific gravity is the point where the proportionality between volume change and weight change ceases. Physically, then, minimum specific gravity is the point where the cellulose of the fibre is saturated and any further absorption of liquid would be putting the liquid, with its solid matter in the case of a resin solution, in the interstices of the material where it is thought to impair the desirable properties of the fibre, particularly its flexibility or pliability.

I prefer to use a waterproofing solution containing 50% Bakelite Water Soluble Resin 25 XR-568 and 50% of water, though a large number of experiments apparently indicate that a dilute solution will waterproof fibre as well as a more concentrated solution. I have also found that the same solution may be used for a considerable length of time, probably due to the fact that the concentration of the solution changes but little during the treatment.

The fibre may be treated with the waterproofing solution at any desired or preferred stage in its 35 manufacture; i. e. before or after the chemicals have been leached or "pured out" or before or after the vulcanized fibre has been dried. As a matter of fact, the process may be applied to completed articles of vulcanized fibre. Extensive 40 experiments indicate that, all other things being equal, a sheet or slab of fibre treated with waterproofing material just after the chemicals have been "pured out" and while the fibre is still thoroughly wet can be rendered considerably more 45 water resistant than an exactly similar sheet or slab of dry fibre. However, I prefer to treat dry fibre for the water of web fibre serves to change the concentration of the waterproofing solution and renders accurate control exceedingly difficult.

At the present time I prefer to immerse the sheets or slabs into tanks or vessels containing the waterproofing solution until the material has absorbed sufficient of the solution to bring its specific gravity down to the minimum. There are 55 various ways of determining the time of immersion. A relatively simple one consists in immersing a small weighed sample of the fibre under treatment in the same waterproofing bath at the same time as the material under treatment 60 and determining its specific gravity at spaced intervals. When the sample or control has reached minimum specific gravity, it is time to remove the material from the bath. Another way is to make test runs with several samples from 65 the batch to determine the length of time necessary to reach minimum specific gravity. By means of test runs on the different types and thicknesses of fibre produced at the plant, a series of charts or graphs may be prepared showing the 70 time of immersion for the different types and thicknesses. Then the time of immersion for any given batch may be readily determined by consulting the appropriate chart or graph.

By immersing sheets of dry fibre in waterproof-

ing solutions of different concentrations, removing them at minimum specific gravity, weighing them, drying, curing and then testing them, it was found that the maximum amount of solid material that could be incorporated in the fibre without altering its desirable physical characteristics was about 10 to 12% by weight. The concentration of the waterproofing bath which yielded this result was a 50% varnish and 50% water solution by volume. This solution has a solid content of 28 gram per gram of liquid, as determined by actual test.

The test used to determine the solid content of the liquid varnish is the standard Bakelite test. It consists in carefully weighing about 5 grams of the varnish mixture in an open dish of about three inches in diameter and then placing it in an oven at 130° C. for three hours, after which time it is cooled and weighed. The weight of the residue left in the dish and the weight of the liquid sample taken are used to compute the percentage of solid matter by weight. The solid matter contained in the finished water resistant fibre is computed as follows: A small piece of the fibre to be treated is first carefully weighed and then immersed in the solution with the sheets which are to be treated. At close intervals it is removed, washed in alcohol to remove the surface film, weighed in air and finally suspended in water to determine its specific gravity. Its weight at minimum specific gravity less the original weight is the weight of the liquid absorbed. The weight of this absorbed liquid multiplied by the per cent solids of this liquid yields the number of grams of solid matter taken up by the fibre. The weight of the solids absorbed divided by the original weight is the percentage of solids contained in the sample. Since the main batch is treated in exactly the same way, it is clear that it contains the same percentage of solids.

Since the foregoing tests indicate that for a 50-50 varnish bath the fibre, if removed at minimum specific gravity, will contain about 10 to 12% of solids by weight, a simple procedure is to remove the batch of material from the impregnating bath when it has taken up about 10% solids. This procedure obviates the necessity for determining specific gravities.

After the fibre is removed from the bath it is washed in alcohol to remove the surface film, dried at 60° C. one or more days, depending upon its thickness, then pressed in a steam heated hydraulic press under a platen pressure of 200 pounds per square inch, at a temperature of 177° C. (125 pounds steam pressure) from ten to twenty minutes depending upon the thickness of the fibre being treated.

The following data is given to prove that the waterproofing treatment does not impair the desirable characteristics of vulcanized fibre:

|                           | 3/16" Red fibre |         | 3/16" White fibre |         |
|---------------------------|-----------------|---------|-------------------|---------|
|                           | Untreated       | Treated | Untreated         | Treated |
| Specific gravity.....     | 1.30            | 1.28    | 1.32              | 1.35    |
| Shearing strength.....    |                 |         |                   |         |
| Lengthwise.....           | 11,000          | 10,950  | 11,000            | 12,950  |
| Crosswise.....            | 11,800          | 13,575  | 13,900            | 15,220  |
| Tensile strength.....     |                 |         |                   |         |
| Lengthwise.....           | 13,300          | 15,420  | 16,550            | 14,950  |
| Crosswise.....            | 8,900           | 10,000  | 8,750             | 9,440   |
| Compressive strength..... | 30,100          | 34,900  | 37,000            | 39,000  |

The foregoing constitutes the essential and distinctive thought of my invention. It is to be understood that its details may be modified in

various ways or combined with various other details without sacrificing any of its advantages. It is to be further understood that the invention is not dependent upon any explanations or theories which have been set forth as descriptive of the actions involved, nor dependent upon the soundness or accuracy of any theoretical statements so advanced. The invention is to be limited solely by the following claims which are to be read in the light of the foregoing description and in which I intend to claim all the novelty inherent in the invention which is permissible in view of the prior art.

In the foregoing description and the following claims the term "paper" is to be understood in its ordinary significance in the art; namely, a sheet or web or cellulosic material from whatever source or sources derived and suitable for the manufacture of indurated fibre. The terms "fibre", "vulcanized fibre" and "indurated fibre" are used interchangeably to denote a cellulosic material so treated chemically and/or physically as to impart thereto a hardness and density not ordinarily possessed by untreated paper. The terms "synthetic resin", "resinoid" and "waterproofing material" are used to denote a synthetic or modified natural resin or equivalent material adapted to permeate or impregnate paper or fibre and decrease its avidity for water.

I claim:

1. A method of increasing the water-resistance of a cellulosic material without impairing its desirable characteristics, which consists in immersing said material in a solution of a synthetic resin in an intermediate stage until the combination of cellulosic material and resin reaches minimum specific gravity and converting said resin to its final stage.

2. A method of increasing the water-resistance of vulcanized fibre without impairing its desirable characteristics, which consists in impregnating said fibre with a water soluble synthetic resin until the combination of fibre and resin reaches minimum specific gravity, drying the material and converting said resin to final insoluble form.

3. A method of increasing the water-resistance of vulcanized fibre without impairing its desirable characteristics, which consists in immersing said fibre in a solution of a synthetic resin in an intermediate stage until the combination of fibre and resin reaches minimum specific gravity, drying the material and converting said resin to final insoluble form.

4. A method of increasing the water-resistance of vulcanized fibre without impairing its desirable characteristics, which consists in immersing said fibre in a solution of a phenol-aldehyde resin in an intermediate stage until the combination of fibre and resin reaches minimum specific gravity, drying the material and converting said resin to final insoluble form.

5. As an article of manufacture, a sheet of substantially flexible, water-resistant material consisting of vulcanized fibre, the fibres of which are substantially saturated with a resinoid and the interstices of which are substantially devoid of resinoid.

6. As an article of manufacture, a sheet of substantially flexible, water-resistant material consisting of vulcanized fibre, the fibres of which are substantially saturated with a resinoid of the phenol-aldehyde type and the interstices of which are substantially devoid of resinoid.